

## UNITED STATES PATENT OFFICE

AUGUST C. ORTHMANN, OF MILWAUKEE, WISCONSIN, ASSIGNOR TO PFISTER & VOGEL LEATHER CO., OF MILWAUKEE, WISCONSIN, A CORPORATION OF WISCONSIN

## UNHAIRING AGENT

No Drawing.

Application filed March 5, 1928. Serial No. 259,388.

The invention relates to leather and more particularly to the treatment of the hide previous to unhairing.

The object of the invention is to provide a new and useful agent for use in facilitating the unhairing of hides. More specifically, I have discovered that beet sugar waste, either as beet sugar molasses or the waste from beet sugar molasses after the removal 10 of all the available sugar therefrom, when treated to render it strongly alkaline will provide an agent far superior to those commonly used for putting the hide in condition for ready removal of the hair therefrom in that the time for preparing the hides is greatly reduced over the methods heretofore known and the hair is in condition for ready removal.

The invention further consists in the several features hereinafter set forth and more particularly defined by claim at the conclusion hereof.

In producing the agent for facilitating unhairing which I will hereafter call the 25 unhairing agent, I take beet sugar waste and render it alkaline by adding a suitable alkali such as caustic soda or lime thereto. By the term beet sugar waste I mean the desugaring waste of the beet sugar 30 process. This desugaring waste is a by-product of the sugar making process and has not been considered heretofore to have much commercial value. I find however, when such beet sugar waste is treated with 35 an alkali to render it alkaline, preferably strongly alkaline and a hide is subjected to a solution of this alkaline beet sugar waste product that the hide is ready for unhairing in less than half the time usually necessary and is in a very favorable condition 40 for hair removal. I attribute this action to the fact that the alkali above described combines with certain constituents of the beet sugar waste to liberate amines which has 45 a marked effect on the tissue surrounding the hair follicles or roots whereby the hair becomes loosened and may be readily removed by the usual unhairing machines or by hand.

50 As a specific example of the manner of

using the unhairing agent above described I take 150 parts of water, 3 to 3½ parts of caustic soda, 8 to 20 parts of beet sugar molasses to 33 parts of weight of hide which has preferably been previously soaked (in 55 water).

The hides are placed in the above solution in a tank or vat and are allowed to soak therein until in a condition for unhairing and during this time the solution may be agitated by suitable mechanical means or the hides may be turned occasionally. I find that following the above formula that hides may be unhaired very satisfactorily after a period of thirty to 60 forty-eight hours at ordinary room temperature which is about 70° Fahrenheit. To hasten the process the solution may be heated to a temperature of about 85° Fahrenheit. During this treatment amines are 65 liberated from the beet sugar waste in an alkaline solution and in the presence of hide so that the liberated amines can act immediately as an unhairing agent. Under 70 the usual process of unhairing hides it requires one hundred and twenty hours or five days' time to put the hides in condition for 75 unhairing.

After the hides have been treated as noted above the solution may be used again 80 to treat a new batch of hides and I have found that the solution may be used several times without necessitating its renewal.

In the case of beet sugar molasses, enough 85 caustic soda is added to provide about a two per cent excess alkaline solution and depending upon the amount of sugar in the molasses I may use from two per cent to five per cent of alkali to one hundred parts of 90 the beet sugar molasses, by weight. Where the beet sugar waste is from beet sugar molasses, after the removal of the sugar therefrom, less alkali needs to be added to render the solution strongly alkaline.

95 Where lime (CaO) is used in place of the caustic soda I use about twenty to thirty pounds of lime to one hundred pounds of the beet sugar waste to obtain the desired alkalinity though this may vary somewhat 100

from the specified amount, depending upon the amount of sugar present in the beet sugar waste. While I have mentioned caustic soda and lime more specifically, it will be understood that I may use potassium hydrate, the carbonates of sodium or potassium, trisodium phosphate, or any other suitable alkali or agent having an alkaline reaction and that I aim to cover these and other variations that may come within the scope of my invention as defined by the claim.

What I claim as my invention is:

As a new unhairing agent for hides, de-sugaring waste from the beet sugar process in a strongly alkaline condition.

In testimony whereof I affix my signature.

AUGUST C. ORTHMANN.

**20**

**25**

**30**

**35**

**40**

**45**

**50**

**55**

**60**

**65**